

Nov. 24, 1931.

W. F. GRUPE

1,833,461

CORK ENVELOPE FOR LAUNDRY ROLLS

Filed June 9, 1924

Fig. 1.



Fig. 2.



Fig. 7.



Fig. 3.



WITNESSES 26

Oliver W. Johnson

Fig. 4.



Fig. 5.



INVENTOR  
William F. Grupe,  
Henry J. Lueke,  
ATTORNEY.

Fig. 6.

## UNITED STATES PATENT OFFICE

WILLIAM F. GRUPE, OF LYNDHURST, NEW JERSEY, ASSIGNOR TO ARMSTRONG CORK COMPANY, OF LANCASTER, PENNSYLVANIA, A CORPORATION OF PENNSYLVANIA

## CORK ENVELOPE FOR LAUNDRY ROLLS

Application filed June 8, 1924. Serial No. 719,009.

This invention relates to envelopes for rolls of mangles and other laundering and similar devices.

An object of the invention is to provide rolls of the above character with a facing of cork in such form of material and of arrangement relative to the body of the roll whereby the envelope provides improved ironing and similar laundering operation.

10 The body of a roll for a mangle and similar laundering and like apparatus is usually of steel of substantially cylindrical form. Heretofore, it has been proposed to surface the cylindrical face with natural cork, applied in 15 assembled form of separate blocks, but such procedure has not been successful by reason of the difficulty of securement of the blocks to the cylindrical face of the roll, and further by reason of such arrangements giving 20 rise inevitably to spaces or clearances in which the steam is entrapped, causing disintegration of natural cork. Such prior procedure is commercially impractical also by reason of the continuous softening and accompanying 25 continuous reduction in effective diameter of the facing of natural cork, due to the pressure arising in the ironing operation.

It has also been heretofore proposed to employ cork particles in the form known as composition cork, wherein albumen, casein or 30 like binding material is employed to bond the cork particles to one another, but such resulting cork facing is defective for laundering operations by reason of the disintegration of the binding material due to chemical action induced under the necessary heat 35 and pressure conditions, and undergoing putrefaction, with attendant physical crumbling and breaking up of the cork particles.

40 Pursuant to the present invention, the cork facing is formed of cork particles bonded to one another under pressure and elevated temperature greatly exceeding the pressure and temperature of laundering conditions and 45 causing the natural resins of the cork to exude to bind the cork particles to one another and resulting in a mass possessing resiliency and other characteristics of such nature most advantageous for laundering purposes; preferably, the envelope is as a complete ring to

encircle the roll, and also extending from end to end of the body of the mangle or other laundering roll. Such cork facing is molded from cork particles and shaped in the mold or the like to have a ring configuration of an inner diameter corresponding to the outer diameter of the body of the roll. 55

Further features and objects of the invention will be more fully understood from the following detail description and the accompanying drawings, in which 60

Fig. 1 is a perspective view of a mangle roll provided with a cork facing embodying my invention; about the improved cork facing are wrapped the usual linen or like fabric 65 cloths;

Fig. 2 is a perspective view of the improved cork facing, shown in Fig. 1;

Fig. 3 is an end elevation of Fig. 2;

Fig. 4 is an end elevation of a modification, 70 of the invention;

Fig. 5 is an end elevation of a further modification of the invention;

Fig. 6 is a detail view on a greatly enlarged scale indicating one manner of structure of 75 cork particles bonded pursuant to my invention; and

Fig. 7 is a similar detail view showing a modified form of bonded structure of cork particles. 80

Referring to Fig. 1, the roll 10 represents the usual or approved form of the body of the roll for a mangle, or laundering machine or the like, usually of steel, and of substantially cylindrical form. Such roll 10 may be 85 mounted on oppositely disposed, central trunnions 12, projecting from the opposite flat end faces 13, 13.

The usual mangle or like laundering machine embodies a set of two or more individual rolls 10, mounted in suitable relation to a steam chest, of steel or the like, (not shown) and formed hollow for the reception of steam or the like heating medium, and usually covered with cloths; the articles to be ironed or otherwise laundered are passed between the set of rolls and the steam chest. 90

About the cylindrical surface 11 of the roll 10 is applied the facing 14 of cork, see Figs. 2 and 3, formed as a ring or annulus prefera- 100

bly extending completely about the cylindrical face, and from one end 13 to the opposite end 13 of the body of the roll 10.

The resulting envelope 14 of cork is re-  
5 movably locked to the cylindrical surface 11  
of the roll 10 by suitable means, as by pro-  
viding the cork envelope 14 with interior  
projections 15 and the cylindrical surface 11  
of the body of the roll 10 with corresponding  
10 slots 16, see Fig. 3. Such projections 15 may  
be formed on the inner face of the cork ring  
14 in uniform spacing and formation, thereby  
providing supplemental to the locking  
15 feature the resilient effect of air cushions  
afforded by the clearances 17 between the  
inner faces of the curved portions 18 of the  
projections 15 and the outer face 11 of the  
body of the roll 10.

As one method of forming the cork facing  
20 or envelope, cork granules or like particles,  
are fed into a suitable mold, such as a two-  
part mold, i. e., a closed outer, female mold  
section and an inner male mold section, and  
the particles progressively fed between the  
25 mold sections, with application of the re-  
quired pressure as by means of a suitable  
tamping tool, to fully fill the mold, and then  
subject the mold and enclosed cork particles  
to an elevated temperature, to effect the  
30 exuding of the natural resins of the cork  
particles through the natural pores of the  
cork particles, and exteriorly of the cork  
particles, whereupon after cooling, the natural  
resins serve as a binding medium for the  
35 cork particles and the cork is transformed  
into a substantially continuous mass of  
substantially homogeneous composition and  
wholly devoid of pores or perforations. The  
resulting binder is insoluble in water and  
40 withstands the temperature and pressure of  
ironing and like laundering operations.

If desired, resins of higher fusion or higher  
plastic point as compared with the resins of  
natural corkwood, may be added to the cork  
45 particles while in the mold.

The usual cloths 19 of linen, or the like, are  
applied to the exterior of the cork facing 14,  
and of a thickness as may be desired.

As auxiliary means for providing the  
50 cushioning effect of the cork facing, the cork  
facing 14 may be molded to have recesses,  
20, see Fig. 4, preferably disposed substan-  
tially uniformly about the exterior surface  
of the cork facing 14. By the heat and pres-  
55 sure treatment of the cork particles while in  
the mold, the inner faces of the recesses 20  
will have become coated with the resins nat-  
ural in the cork or as added in the molding  
stage, thereby coating the inner faces of the  
60 recesses 20 with a steam and moisture resist-  
ant envelope.

In Fig. 4, I have shown a modification of  
the invention wherein the inner face of the  
cork ring 14 is fluted or corrugated, as in-  
65 dicated at 21, for engagement with the outer

face 11 of the body of the roll 10; between  
the inner faces 22 of the flutings and the roll  
are provided clearances serving as cushions.

In Fig. 5, the cork ring 14 is formed simi-  
larly as hereinabove described, and provid-  
ed with a substantially cylindrical outer fac-  
ing 23 and a substantially cylindrical inner  
facing 24; the diameter of the inner facing  
24 is preferably such as to make a substan-  
tially tight fit with the outer cylindrical fac-  
ing 11 of the body of the roll 10; to enhance  
the locking of the cork envelope 14 of the  
form shown in Fig. 5, relative to the cylind-  
rical face 11 of the body of the roll 10, a  
70 key-slot 25 may be molded or cut on the in-  
ner face 24 of the cork ring 14, for receiving  
a wedge of steel or like material, positioned  
under pressure.

If desired, the ring of the form shown in  
Fig. 5, may be provided with exteriorly dis-  
posed recesses, such as the recesses 20 shown  
in the modification of Fig. 4.

The cork facing or envelope produced in  
accordance with my invention may be ap-  
plied as a number of sections, in end to end  
engagement about the periphery of the roll,  
and may be of semi-cylindrical as indicated  
at 26, quadra-cylindrical or like sectional  
formations.

Preferably, the treatment of the cork par-  
ticles is carried out at a temperature of up-  
wards of 500° Fahrenheit and at a pressure  
sufficient to effect the bonding of the cork  
particles to one another. The pressure of  
the bonding treatment may be varied in cor-  
respondence to the desired degree of hard-  
ness and resiliency of the resulting product;  
as an example, the cork particles may be com-  
pressed in the treating mold from a volume  
of, say, three to a volume of unity.

At ordinary temperatures, the resulting  
cork facing or envelope is relatively hard  
and readily withstands shipment and the  
comparatively severe handling in installa-  
tion on the laundering roll.

By greater reduction of volume of the  
treated cork particles, the degree of hard-  
ness of the resulting cork mass may be in-  
creased; and, correspondingly, by decreased  
reduction of volume of the treated cork par-  
ticles, the degree of hardness of the result-  
ing cork mass is decreased.

At the temperature of ironing or like laun-  
dering operation, usually approximately  
250° Fahrenheit, the cork facing or envelope  
possesses most admirable qualities for effect-  
ing smooth ironing notwithstanding vary-  
ing thicknesses of the laundered materials.  
At the ironing temperature, the cork mass  
accommodates itself at all times to abrupt  
120 changes of thickness of laundered material  
due to the presence of buttons or like ad-  
denda of relatively hard material, thereby  
avoiding damage to the same, and is most  
effective in emphasizing raised or relief or-  
125 130

namentation of laundered material, such as embroidered tablecloths, bed coverings and the like.

The above noted nature of flexing resiliency at ironing temperatures and comparative hardness at ordinary temperature are more advantageously attained by the use of flat particles of cork of varying superficial areas and of a thinness of the magnitude of ordinary paper; such thin particles 27, see Fig. 6, are assembled and bonded in the resulting mass 28 in more or less overlapping relation to one another.

In a similar manner, cork particles derived by "grinding" so-called tapered cork waste, resulting in the manufacture of tapered corks and comprising flat shavings of tapered thicknesses may be employed pursuant to my invention to yield a cork mass of interlocked flat particles varying in thickness from that of ordinary paper to that of cardboard.

Upon feeding such cork particles of flat formation into a mold of the type referred to hereinabove, and disposing the outer and inner mold sections with their longitudinal axes extending substantially vertically, and compressing the same by tamping and subjecting the same to the baking temperature as hereinabove described, the resulting mass is constituted of cork particles 27 bonded to one another with their flat faces in overlapping relation extending substantially radially with respect to the center of the molded cork envelope or facing 28, as indicated generally in Fig. 6. Accordingly, the resisting compression within the cork particles arising in the ironing operation is directed in planes substantially parallel to the flat faces of the interbonded cork particles.

In Fig. 7, I have illustrated a portion of an envelope or padding 30 formed pursuant to my invention from a mixture of relatively thick particles 31 and thin particles 32, as by intermixing granular cork waste or ground cork disk waste with "ground" cork flakes in varying proportions; in such instances, the thin particles 32 interbond the thereby flattened relatively thick cork particles 31 as well interbond one another. Such result may be attained with an intermixture of cork particles having thicknesses varying from that of tissue paper for the thin particles 32 to cardboard for the relatively thick particles 31, or a range of from ten to unity in relative thicknesses.

It will be observed that in the tamping or like compression operation preliminary to the baking treatment, the relatively thick cork particles are compressed irrespective of location in the mass, in the direction parallel to the direction of length or axes of the mold, that is to say, substantially at right angles to the direction of compression arising in the ironing or other laundering operation. Such

relation of compression of all particles in the cork padding preserves fully freedom of the resiliency of the cork particles under ironing conditions in the direction substantially parallel to their direction of length, i. e., parallel to their flat faces, and it is my belief that the superior nature of resiliency attending the state of comparative softness of the cork padding at ironing temperatures is ascribable to such relation of the compression between the cork particles effected in the baking treatment.

If desired, the cork padding may be of sheet form and wound about the ironing or other laundering roll to attain the desired effective diameter.

To form such sheet of cork padding pursuant to my invention, the cork particles preferably of flake form are laid upon another, the flat faces thereof being positioned in more or less overlapping relation to one another; and thereupon, the mass of cork particles are compressed under minimum pressure represented by the reduction in volume from four to one and then baked similarly as hereinabove described to the molded cylindrical form.

The mass is bonded as a whole by the resins distributed more or less through the mass in the baking stage. However, the bonding between the cork particles is not continuous between the cork particles, but at spaced points, thereby giving rise to intervening relation non-bonded areas and consequent air spaces. Accordingly, under the ironing or similar laundering conditions, such nature of interbonding permits the cork particles to be flexed relatively to one another, which action is enhanced by the intervening cushioned air.

Padding formed pursuant to my invention is also applicable to ironing and other laundering machines of the so-called flat bed type, for which use the cork padding is molded in flat formation. In the forming of such flat cork padding, the particles are fed into a suitable mold in the direction of length of the mold, the mold being positioned vertically with respect to its length to thereby locate the particles with their faces of greatest area to extend substantially horizontally; and then compressed vertically; the baking resulting in exuding the resins is carried out similarly as hereinabove described.

It will be noted that in the substantially flat padding type, the cork flakes are similarly interbonded at spaced areas with one another or with the flattened thicker cork particles, and with the flat faces of all particles extend substantially in the direction of thickness of the cork padding. Such formation of flat cork padding, bonded as a whole by interbonding of the cork particles at spaced areas and intervening non-bonded areas and air spaces between the particles, is highly adapted for flat bed laundering machines,

such as for pressing cloth, garments and like articles, in which the heat is produced by steam applied at the bottom of and transmitted through the cork padding, and the articles are pressed over the top of the cork padding whereby the vertical positioning and the above referred to nature of inter-bonding of the cork particles enhance the conduction of the steam and heat through the cork padding.

Such vertical positioning of the cork particles interiorly of the flat cork padding facilitates discharge from the padding of steam or moisture from the cloth, garments or like articles generated by the pressing operation, thereby "enlivening" the cork particles, as I have discovered, and minimizing any tendency towards charring.

Whereas I have described my invention by reference to specific forms thereof, it will be understood that many changes and modifications may be made without departing from the spirit of the invention.

I claim:

1. An envelope for rolls of mangles and the like and subject to laundering temperatures of 212° F., comprising a mass of inherently flat cork particles bound to one another by resins natural in cork, said envelope extending substantially continuously about the periphery of the roll.

2. An envelope for rolls of mangles and the like and subject to laundering temperatures of 212° F., comprising a mass of inherently flat cork particles bound to one another by resins natural in cork, said envelope extending substantially continuously about the periphery of the roll and substantially continuously from end to end of the roll and means for removably locking the cork envelope to the roll.

3. An envelope for rolls of mangles and the like and subject to laundering temperatures of 212° F., comprising a mass of inherently flat cork particles bound to one another by resins natural in cork, said envelope extending substantially continuously about the periphery of the roll and means distributed on the inner face of the cork envelope for removably locking the same to the roll.

4. A padding for laundering machines and subject to laundering temperatures of 212° F. comprising a mass of inherently flat cork particles bonded to one another under temperature and pressure conditions respectively materially exceeding the maximum temperature and maximum pressure of laundering operations.

5. A padding for laundering machines and subject to laundering temperatures of 212° F. comprising a mass of inherently flat cork particles bonded to one another under temperature and pressure conditions respectively materially exceeding the aforesaid laundering temperature and the maximum pressure

of laundering operations, and possessing resilience and substantial permanence of dimensions under laundering conditions.

6. A padding for laundering machines and subject to laundering temperatures of 212° F. comprising a mass of cork particles of inherently substantially flat formation bonded to one another under pressure and at a temperature materially exceeding 300° Fahrenheit.

7. A padding for laundering machines and subject to laundering temperatures of 212° F. comprising a mass of cork particles of inherently substantially flat formation and bonded under pressure in overlapping relation to one another by resinous bonding material.

8. A padding for laundering machines and subject to laundering temperatures of 212° F. comprising a mass of cork particles of inherently substantially flat formation bonded to one another to be disposed with their flat faces substantially parallel to one another and under pressure and at a temperature materially exceeding 300° Fahrenheit.

9. A facing for rolls for laundering machines and subject to the temperature of 212° F. comprising a mass of cork particles of inherently substantially flat formation bonded under pressure to one another to be disposed in planes substantially radially and substantially at right angles to the axis of the roll and at a temperature materially exceeding 300° Fahrenheit.

In testimony whereof I have signed this specification this 3rd day of June, 1924.

WILLIAM F. GRUPE.

105

110

115

120

125

130